

# United States Patent [19]

Demoures et al.

[11] 3,862,981

[45] Jan. 28, 1975

[54] **NEW LUBRICATING OIL ADDITIVES**

[75] Inventors: **Bernard Demoures**, Puteaux; **Daniel Llauro**, Crepieux Le Pape; **Francois Giolito**, Lyon, all of France

[73] Assignee: **Rhone-Progil**, Paris, France

[22] Filed: June 28, 1972

[21] Appl. No.: 267,048

3,522,179 7/1970 Le Suer..... 252/51.5 A  
3,620,977 11/1971 Honnen et al. .... 252/51.5 A

Primary Examiner—Paul F. Shaver

[30] **Foreign Application Priority Data**

July 8, 1971 France ..... 71/26025

[52] **U.S. Cl.** 260/479 S, 44/71, 252/51.5 A

[51] **Int. Cl.** C07c 69/00, C01m 3/26

[58] **Field of Search**..... 260/479 R, 479 S; 252/51.5 A

[56] **References Cited**

UNITED STATES PATENTS

3,278,550 10/1966 Norman et al. .... 252/51.5 A

[57] **ABSTRACT**

New lubricating oil additives are provided comprising the reaction product of diphenylolpropane with an aliphatic chain substituted-succinic anhydride or acid, which aliphatic chain substituent is substantially saturated and contains at least about 30 carbon atoms, said reaction product being neutralized with an amine, preferably a polyamine, such as a polyalkylene-polyamine. Lubricating oils, fuel oils, and carburants containing the new additives have excellent detergent, dispersing and anti-rust properties.

8 Claims, No Drawings

## NEW LUBRICATING OIL ADDITIVES

## BACKGROUND OF THE INVENTION

The present invention relates to new lubricating oil additives which impart to lubricating oils good detergent, dispersing and anti-rust properties. This invention relates also to lubricating oils and to fuels and carburants containing said additives.

There are known to the prior art, additives for lubricating oils which consist of derivatives of succinic acid or anhydride substituted with slightly unsaturated hydrocarbons. This class of additives, which has been known for some years, was an important development to the lubricating oil art. They consist mainly of reaction products of succinic acylating agents, substituted with a fairly saturated hydrocarbon radical containing an aliphatic chain of at least about 50 carbon atoms, with amines or alcohols.

Though the performances of such prior art additives are acceptable, it is desirable and even necessary to improve them. Those additives of the prior art which are esters have deficiencies with regard to their behavior to high temperatures and to their lack of resistance to hydrolysis. The esters are good anti-rust agents, but they have a limited dispersing power. Those additives which are aminated derivatives are good ashless dispersing agents, but they possess poor anti-rust properties.

It is an object of the present invention to provide a lubricating oil additive which does not have the shortcomings of the prior art additives.

It is also an object of the present invention to provide lubricating oils containing the new additives and which oils have improved dispersing, detergent and anti-rust properties.

Another object of the present invention is the provision of a lubricating oil additive having improved properties over those of the prior art alkyl substituted succinic esters described, for example, in U.S. Pat. No. 3,381,022 granted Apr. 30, 1968, and also with regard to the amide derivatives described in U.S. Pat. No. 3,172,892 of Mar. 9, 1965.

Other objects of the invention will be apparent to those skilled in the art from the present description.

## GENERAL DESCRIPTION OF THE INVENTION

The lubricating oil additives of the present invention comprise reaction products of diphenylopropane with an hydrocarbon chain substituted succinic anhydride or acid, which hydrocarbon chain substituent is substantially saturated and contains at least 30 and preferably at least 50, carbon atoms, said resulting product being then neutralized with a polyamine, such as a polyalkylenepolyamine. After an extensive research investigation it has been found that these additives impart improved detergency, dispersing and anti-rust properties to lubricating oils, fuel oils and carburants.

These novel additives and products of the invention are produced in the form of a complex mixture, rather than a precise chemical compound, of which it is difficult to determine the exact chemical composition and the relative proportions present of the various constituents. It is for this reason that the products must be described in terms of the process of manufacturing them. The presence of the ester grouping resulting from the reaction of the diphenylopropane and the substituted succinic anhydride or acid has been confirmed by infrared analysis. The esterification reaction between the

substituted succinic acid or anhydride and diphenylopropane results in an equilibrium difficult to displace; the resulting product contains in solution a variable proportion of the unreacted succinic acylating agent and, as a dispersion in said solution, unreacted diphenylopropane. It is essential, in order to obtain good dispersing properties when employing the product as a lubricating oil additive, to neutralize the unreacted acylating agent with an amino compound. The unreacted diphenylopropane may be removed, if it is in a large excess, by any convenient way such as filtration, centrifugation, etc.

The hydrocarbon chain-substituted succinic acid or anhydride starting materials used in the present invention are those resulting from the reaction of maleic acid or anhydride with a polyolefin, such as polyethylene, polypropylene, polybutylene, polyisobutylene, etc. having a molecular weight sufficient to provide a carbon content of at least about 30 atoms, preferably at least about 50 carbon atoms. The hydrocarbon chain is preferably aliphatic in nature. As a practical matter, the molecular weight of such polyolefins is at least about 400. It is also possible to use a chlorinated polyolefin, such as chloropolyethylene, which is reacted with maleic acid or anhydride. All that is necessary is to react the maleic anhydride with the polyolefin or chlorinated polyolefin at a temperature of between about 150° and 250°C. The reaction product is the polyolefin-substituted succinic anhydride. The substantially saturated hydrocarbon substituent of the succinic radical may contain polar groups in minor proportions: chloro, nitro, etc. Hydrolysis of this product by water or steam treatment will produce the corresponding succinic acid.

The esterification reaction of diphenylopropane with the aliphatic substituted succinic anhydride or acid may be achieved in the presence of a classical esterification catalyst, i.e., a base or acid, such as pyridine or its hydrochloride, sulfuric acid, para-toluenesulfonic acid and ion exchange resins having a strongly or moderately acid character. It may also be achieved without any catalyst. This esterification reaction occurs preferably at a temperature from about 50° to 300°C., preferably between about 100° and 200°C., with or without a solvent such as xylene, toluene, etc. The solvent simplifies both temperature control and water removal from the reaction mixture.

The relative proportions of the two constituents, diphenylopropane and aliphatic substituted succinic acid or anhydride, may vary within large limits. But in any event, since esterification is usually not complete, the remaining acid or anhydride must afterwards be neutralized with an aminated compound. Such neutralization is an important feature of the invention, as it is necessary to obtain good dispersing properties. The unreacted diphenylopropane, finely dispersed in the product resulting from the esterification reaction, may be removed if it is in a substantial quantity. Otherwise it may remain in the product in a divided form without involving any disadvantage or incompatibility.

The esterification reaction involves a time duration of between about 1 and 10 hours, preferably 2 to 6 hours. It may occur under the normal atmospheric pressure, or under an elevated or reduced pressure, or in an atmosphere of inert gas.

The unreacted substituted succinic acid or anhydride present in the product resulting from esterification is

neutralized afterwards by an aminated compound. Among those compounds, a preferred class is the polyamines, including the polyalkylenepolyamines, such as diethylenetriamine, triethylenetetramine, tetraethylenepentamine, pentaethylenhexamine, etc. Others may, of course, also be used.

#### DETAILED DESCRIPTION OF THE INVENTION

In order to disclose more clearly the nature of the present invention, the following examples illustrating the invention are given. It should be understood, however, that this is done solely by way of example and is intended neither to delineate the scope of the invention nor limit the ambit of the appended claims. In the examples which follow, and through the specification, the quantities of material are expressed in terms of parts by weight, unless otherwise specified. The acylating agent used in Examples 1 to 6 hereinbelow is the reaction product of 350 grams of maleic anhydride and 2500 grams of polyisobutene with a molecular weight equal to about 1000.

#### EXAMPLE 1

2 kilograms of polyisobutylene substituted-succinic anhydride, prepared as hereinabove [Pibsa index = 53 - Pibsa index (for polyisobutyl succinic anhydride) is the number of potash milligrams which are necessary for neutralizing 1 gram of product] were reacted with 107 grams of diphenyol propane in the presence of 21 grams of p-toluenesulfonic acid catalyst for 4 hours at a temperature of 160°C. The product was then vaporized under vacuum at 160°C. for 1 hour, and neutralized with 82 grams of tetraethylenepentamine at 155°C. for 2 hours, under a partial vacuum (400 mm. Hg. pressure, approximately). This treatment was followed with a vaporization at 20 mm. Hg. pressure for 30 minutes. Nitrogen content in the final product was 1.29%.

#### EXAMPLE 2

62.5 grams of diphenyolpropane were heated at 170°C. 484 grams of polyisobutylene substituted-succinic acid prepared as hereinabove (Pibsa Index = 63.5) were introduced over 15 minutes at 170°C. under 400 mm. Hg. pressure. The reaction proceeded for 4 hours (170°C. under partial vacuum). 543 grams of the resulting product were treated afterwards with 21.5 grams of tetraethylenepentamine under the same conditions as in Example 1. Nitrogen content in final product was 1.40%.

#### EXAMPLE 3

64 grams of diphenyolpropane were heated in the presence of 472 grams of xylene at 110°-115°C. Then 1257 grams of polyisobutylene substituted-succinic anhydride prepared as hereinabove, (Pibsa Index = 62.5), were introduced over a period of 25 minutes. After 1 hour of reaction at 110°-115°C., 13.2 grams of pyridine were added. A second addition of an equal amount of pyridine was made after 2 hours of reaction. After 3.5 hours of reaction, the product is vapourized at 140°C. under 20 mm. Hg. pressure for 30 minutes.

#### EXAMPLE 4

200 grams of the product of Example 3 were neutralized with 5.6 grams of tetraethylenepentamine under the same conditions as in Example 1. Nitrogen content of the final product was 1%.

#### EXAMPLE 5

200 grams of the product of Example 3 were neutralized with 7.7 grams of triethylenetetramine under the same conditions as in Example 1. Nitrogen content of the final product was 1.42%.

#### EXAMPLE 6

15 6640 grams of polyisobutylene substituted-succinic anhydride (Pibsa Index = 76.3) were reacted with 465 grams of diphenyolpropane in the presence of 53 grams of para-toluene sulfonic acid for 2.5 hours at 162.5°C. Then the product was vapourized under vacuum for 1.5 hours. 667 g. of the resulting product were neutralized with 23.1 grams of tetraethylenepentamine under the same conditions as in Example 1. Nitrogen content of the final product obtained in this way was 1.23%.

#### EXAMPLE 7

30 The acylating agent employed in this example was the reaction product of maleic anhydride with a polyisobutene having a molecular weight equal to about 455, heated at a temperature between 190° and 240°C. for 10 hours.

35 200 grams of the resulting polyisobutylene substituted-succinic anhydride (Pibsa Index = 81) were reacted with 16.46 grams of diphenyolpropane and 2.1 grams of p-tolene-sulfonic acid over 4 hours at 170°C. and for 30 minutes under vacuum at 170°C. 201 grams of the resulting product were reacted with 9 grams of tetraethylenepentamine at 155°C. for 2 hours under partial vacuum (about 400 mm. Hg. pressure). Treatment was completed under vacuum of 20 mm. Hg. pressure for 30 minutes. Nitrogen content of the final product was 1.44%.

40 It will be apparent that in the foregoing examples other polyolefin substituted succinic anhydrides may be employed such as those of polyethylene, polypropylene and polypentene, etc. Also, the amine employed for neutralization may be diethylenetriamine or pentaethylenhexamine, etc.

45 50 The additive products of the invention, including the products of the foregoing examples, are desirably employed in lubricating oils, fuel oils and carburants, in amounts of between about 0.01 and 10%, preferably between 0.1 and 3%, by weight of oil.

55 The foregoing products according to the present invention were tested with regard to anti-rust and dispersing properties in lubricating agents.

60 65 The tests of the dispersing power were conducted according to the stain method described in Volume 1 of A. Schilling's book "Les huiles pour moteurs et le graissage des moteurs" (Oils for motors and motor greasing), edition of 1962, pages 89-90. Stains were achieved with the additive dissolved in a lubricating oil of SAE 30. Sludge was added in order to obtain a content of carbonaceous substances of 0.36%. There are five stains obtained:

1. after heating at 200°C. for 10 minutes
2. after heating at 250°C. for 10 minutes

3. after heating at 200°C. for 10 minutes (at the outset 1% of water was added)
4. after heating at 200°C. during 1 minute (initially 1% of water was added)
5. after adding of 1% of water, in the cold state

Readings were made after 48 hours. For every stain, the dispersed sludge percentage is expressed with regard to the oil stain and calculated from the respective diameters. The higher the percentages of dispersed product; the better is the dispersion with regard to sludge.

For the products in accordance with the present invention of the foregoing examples the following values were obtained:

Example 1 product = 308

Example 2 product = 306

Example 4 product = 301

Example 5 product = 312

A comparison was made of the dispersing values obtained by the same test method with other products such as a non-neutralized ester and prior products commonly used, considered as typical of the present state of the art. Listed below are the values obtained:

|                                                        |      |
|--------------------------------------------------------|------|
| Product of Example 3 (non-neutralized product)         | <200 |
| Monosuccinimide                                        | 268  |
| Bis succinimide                                        | 274  |
| Ester of substituted succinic acid and pentaerythritol | 265  |
| Ester of substituted succinic acid and glycerol        | 250  |
| Ester of substituted succinic acid and phenol          | <200 |

The mono and bis succinimides were tested, on the basis of the same nitrogen content as the products of Examples 1, 2, 4 and 5 (reference: 1% monosuccinimide in SAE 30 oil).

The various prior art succinimide esters listed in the above table were synthesized according to classical esterification processes described hereinbelow and tested, for the same weight as the products of Examples 1, 2, 4 and 5. (1.8% in SAE 30 oil).

#### MONOSUCCINIMIDE PREPARATION

250 grams of polyisobutylene substituted-succinic anhydride having a Pibsa index = 53 were reacted with 18 grams of tetraethylenepentamine at 155°C. for 2 hours, under partial vacuum (about 400 mm. Hg. pressure). Treatment was followed with a vapourization under 20 mm. Hg. pressure for 30 minutes. Nitrogen content of the final product was 2.46%.

#### BIS-SUCCINIMIDE PREPARATION

250 grams of polyisobutylene substituted-succinic anhydride having a Pibsa index = 55 were reacted with 8.6 grams of triethylenetetramine at 155°C. for 2 hours, under a partial vacuum (about 400 mm. Hg. pressure). Treatment was followed by a vapourization under 20 mm. Hg. pressure for 30 minutes. Nitrogen content of the final product was 1.32%.

#### PREPARATION OF SUBSTITUTED SUCCINIC ACID AND PENTAERYTHRITOL ESTER

1258 grams of polyisobutylene substituted-succinic anhydride (Pibsa index = 62.5) were reacted with 94 grams of pentaerythritol for 3.5 hours at 135°-145°C.

then for 2 hours at 175°-185°C. Unreacted pentaerythritol was removed by filtration. The filtrate constituted ester.

#### PREPARATION OF GLYCEROL AND SUBSTITUTED SUCCINIC ANHYDRIDE ESTER

898 grams of polyisobutylene substituted-succinic anhydride with a Pibsa Index = 62.5 were reacted with 46 grams of glycerol for 3 hours at 150°C., then for 3 hours at 190°C. The reaction product was the desired ester.

#### PREPARATION OF PHENOL AND SUBSTITUTED SUCCINIC ACID ESTER

15 898 grams of polyisobutylene substituted-succinic anhydride with a Pibsa index = 62.5 were reacted with 376 grams of phenol in the presence of 190 grams of xylene for 1 hour at 160°-165°C. Afterwards 12.7 grams of p-toluene sulfonic acid were added. The reaction proceeded for 30 minutes at 160°-165°C. This operation was repeated twice. Finally, xylene, residual phenol and catalyst were removed under vacuum (160°-165°C. during 30 minutes — 10 to 20 mm. Hg. pressure). The final product was the ester.

20 The anti-rust characteristics of the products according to the invention have been tested in the laboratory with favorable results. The general tendency has been confirmed by motor tests (sequence II B, gasoline motor V-8 of a 1967 Oldsmobile). The basic formulation to which the additive was added was composed of a calcium sulfonate, a calcium phenate and a zinc dithiophosphate. The following values expressing average engine rust (AER), were obtained (ideal value 10):

25 Basic formula plus Example 1 product — AER 8.6  
Basic formula plus Example 5 product — AER 7.9  
As a comparison of the prior art, the following value was obtained:

30 Basic formula plus bis succinimide — AER 7.2  
The entirety of the test results set forth hereinabove shows quite well the important improvement provided by the additives for lubricating oils produced according to the invention and characterizes the technical progress that such new products have achieved.

35 The terms and expressions which have been employed are used as terms of description and not of limitation, and there is no intention in the use of such terms and expressions of excluding any equivalents of the features shown and described or portions thereof, but it is recognized that various modifications are possible within the scope of the invention claimed.

40 What is claimed is:

1. An additive consisting of the ester reaction product of diphenylopropane with an hydrocarbon substituted-succinic anhydride or acid, wherein the said hydrocarbon substituent is substantially saturated and contains at least about 30 carbon atoms, said reaction product being neutralized with a polyamine.

45 2. An additive in accordance with claim 1, wherein said polyamine is a polyalkylenepolyamine.

3. An additive in accordance with claim 2, wherein said polyalkylenepolyamine is a member selected from the class consisting of diethylenetriamine, triethylenetetramine, tetraethylenepentamine and pentaethylenhexamine.

50 4. An additive in accordance with claim 1, wherein said hydrocarbon substituent is a polyolefin radical.

5. An additive in accordance with claim 1, wherein said hydrocarbon substituent is a chlorinated polyolefin radical.

6. An additive in accordance with claim 1, wherein said hydrocarbon substituent contains at least about 50 carbon atoms.

7. An additive in accordance with claim 4, wherein said polyolefin radical is derived from a member of the

class consisting of polyethylene, polypropylene, polybutylene, polyisobutylene, polypentene-1 and chlorinated polyolefins.

5 8. An additive in accordance with claim 1, wherein the esterification reaction is conducted at a temperature of between about 50° and 300°C.

\* \* \* \* \*

10

15

20

25

30

35

40

45

50

55

60

65